

## UNITED STATES PATENT OFFICE

2,103,497

ARTIFICIAL TEXTILE MATERIAL AND  
METHOD OF PREPARING THE SAMEGeorge Schneider, Montclair, N. J., assignor to  
Celanese Corporation of America, a corpora-  
tion of DelawareNo Drawing. Original application May 4, 1934,  
Serial No. 723,844. Divided and this applica-  
tion June 10, 1936, Serial No. 34,479

18 Claims. (Cl. 28—1)

This invention relates to the preparation or treatment of artificial materials particularly textile materials, such as yarns or filaments made of organic derivatives of cellulose, whereby the same are rendered more amenable to textile operations or have other improved properties.

This application is a division of my application S. No. 723,844 filed May 4, 1934.

An object of my invention is to prepare or treat textile materials, particularly yarns or filaments containing cellulose acetate or other organic derivatives of cellulose by the employment of oils or fatty acids in conjunction with a para-benzene derivative, whereby the yarns or filaments are rendered more pliable and can therefore be knitted, woven or knotted more readily. Other objects of the invention will appear from the following detailed description.

It is desirable to apply finishes which soften or lubricate the yarns in many processes of conversion of textile yarns such as twisting, winding, knitting or weaving. The finishes considered most useful for this purpose contain oils, such as olive oil or castor oil. However, when such oils are applied to the yarn, upon ageing they hydrolyze to develop free acid; they tend to oxidize and to polymerize and form viscous and gummy bodies.

I have found that if para-benzene derivatives containing an OH radicle are added to such oils, yarns to which the resulting mixture has been applied, remain soft and not sticky when exposed to the air for long periods of time. Moreover the presence of these para-benzene derivatives greatly retard the development in such oils of free acidity, prevent oxidation and largely overcome the tendency of such oils upon ageing to render cellulose acetate yarns less resistant to the delustering action of hot aqueous liquids. All phenol derivatives have some preservative power in oils. I have found, however, that outstanding in effectiveness in this respect, are the para derivatives of phenol such as hydroquinone.

In accordance with my invention I employ the animal or vegetable oils or the fatty acids derived therefrom in conjunction with para derivatives of phenol in the preparation or treatment of artificial materials particularly those contain-

ing cellulose acetate or other organic derivatives of cellulose.

The animal or vegetable oils employed may be any suitable one such as olive oil, teesed oil, peanut oil, castor oil, cocoanut oil, neatsfoot oil and in general the glycerides of the higher fatty acids such as oleic acid, palmitic acid or stearic acid. One of such oils or a mixture of two or more such oils may be employed. If desired the fatty acids themselves may be employed. These oils may be used alone or in conjunction with mineral lubricating oils and sulphonated oils as well as in conjunction with bodies having a beneficial effect such as diethylene glycol, glycerine, etc.

In order to prevent such oils and fatty acids from oxidizing, hydrolyzing, polymerizing or otherwise becoming sticky and thus imparting harshness to the textile material, I add a para derivative of phenol. Any suitable para derivative of phenol may be employed, for example hydroquinone, methyl ester of paraoxy benzoic acid, propyl ester of paraoxy benzoic acid and other like derivatives of benzol. The para derivatives of benzene may have the graphic formula



where R is OH or COOR<sup>1</sup> wherein R<sup>1</sup> is an alkyl group such as methyl, ethyl, butyl and propyl radicals.

The amount of para derivative of phenol employed may be any suitable one being usually small and on the order of 0.2 to 4% of the weight of the oils or fatty acids employed.

In one form of my invention, the vegetable or animal oils or the fatty acids in admixture with the para derivative of benzol may be added to the spinning dope or solution from which the yarns, filaments, artificial bristles or straw and the like are formed, and such solution may then be extruded through orifices to an evaporative atmosphere as in dry spinning or into the precipitating bath as in wet spinning, or thin foils or thin films may be made from such solutions by casting the same on to a film casting wheel or by other known methods.

In another form of my invention the mixture of oils or fatty acids and the para derivative of phenol may be applied to the yarns, filaments, fabrics, films or foils after their formation. They 5 may be applied either alone or in admixture with other materials as a lubricant or finish. Thus the lubricant or finish may also contain softening agents such as the polyhydric alcohols, their derivatives and substitution products, the 10 examples of which are diethylene glycol and glycerine.

The textile materials or other artificial materials to be prepared or treated in accordance with this invention preferably contain organic 15 derivatives of cellulose which may be organic esters of cellulose or cellulose ethers. Examples of such organic esters of cellulose are cellulose acetate, cellulose formate, cellulose propionate and cellulose butyrate, while examples of such 20 cellulose ethers are ethyl cellulose, methyl cellulose and benzyl cellulose.

Yarns, artificial straw or filaments when prepared or treated in accordance with this invention have great pliability due to the presence of 25 the animal or vegetable oils or the free fatty acids, as shown by the fact that such yarns may be readily knitted into fabric containing many stitches per unit length and artificial bristles, horsehair and straw may be knotted quite tightly 30 and bent quite severely without breaking. Moreover when such yarns are exposed to the air for long periods of time, because of the presence of the para derivative of phenol, they retain their softness and pliability and can be readily knitted. 35 In order to further illustrate my invention but without being limited thereto the following specific example is given.

*Example*

40 A finish is prepared as follows:

Olive oil----- 99 parts by weight  
Para derivative of phenol--- 1 part by weight

45 In the above mixture, the para derivative of phenol may be the methyl ester of parahydroxy benzoic acid, or the propyl ester of parahydroxy benzoic acid. The above mixture is applied to a yarn consisting wholly of acetone soluble cellulose acetate filaments, by causing such yarn to pass over wicks, rollers or other furnishing devices for applying such mixture, in their transit from the dry spinning machine in which they are 50 formed to a winding device. The amount of finish applied is from 1 to 6% on the weight of 55 the yarn.

The para derivatives of phenol greatly reduce the tendency of the olive oil to polymerize upon ageing and inhibits oxidation. Moreover while 60 cellulose acetate yarns or fabrics treated with olive oil alone after a period of time tend to deluster more readily when treated with hot aqueous fluids the presence of the para derivative of phenol greatly reduces this tendency of delustering. 65 Moreover, the above type of finish has the property of maintaining a finish, over the entire yarn or fabric, of the same consistency. Thus when the material is subjected to dyeing, washing or other hot aqueous liquid treatments there 70 is no streakiness produced as in the case where the lubricant finish tends to change its chemical composition in one place more than in another.

75 It is to be understood that the foregoing description is given merely by way of illustration, and that many variations may be made therein,

without departing from the spirit of my invention.

Having described my invention, what I desire to secure by Letters Patent is:

1. Process of improving the properties of filaments or yarns containing organic derivatives of cellulose comprising applying thereto a finish containing a fatty material selected from the group consisting of higher fatty acids and their glycerides and an alkyl ester of a para hydroxy 10 benzoic acid. 5

2. Process of improving the properties of filaments or yarns containing cellulose acetate comprising applying thereto a finish containing a fatty material selected from the group consisting of higher fatty acids and their glycerides and an alkyl ester of a para hydroxy benzoic acid. 15

3. Process of improving the properties of filaments or yarns containing organic derivatives of cellulose comprising applying thereto a finish 20 containing a glyceride of a higher fatty acid and an alkyl ester of para hydroxy benzoic acid.

4. Process of improving the properties of filaments or yarns containing cellulose acetate comprising applying thereto a finish containing a 25 glyceride of a higher fatty acid and an alkyl ester of para hydroxy benzoic acid.

5. Process of improving the properties of filaments or yarns of cellulose acetate comprising applying thereto a finish containing olive oil and an 30 alkyl ester of para hydroxy benzoic acid.

6. Process of improving the properties of filaments or yarns of cellulose acetate comprising applying thereto a finish containing olive oil and the methyl ester of para hydroxy benzoic acid. 35

7. Process of improving the properties of filaments or yarns of cellulose acetate comprising applying thereto a finish containing olive oil and the propyl ester of para hydroxy benzoic acid.

8. Artificial material of organic derivatives of 40 cellulose containing a fatty material selected from the group consisting of higher fatty acids and their glycerides and an alkyl ester of a para hydroxy benzoic acid.

9. Artificial material of cellulose acetate containing a fatty material selected from the group 45 consisting of higher fatty acids and their glycerides and an alkyl ester of a para hydroxy benzoic acid.

10. Artificial yarns and filaments of organic 50 derivatives of cellulose containing a glyceride of a higher fatty acid and an alkyl ester of para hydroxy benzoic acid.

11. Artificial yarns and filaments of cellulose acetate containing a glyceride of a higher fatty 55 acid and an alkyl ester of para hydroxy benzoic acid.

12. Artificial yarns and filaments of cellulose acetate containing a vegetable oil and an alkyl ester of para hydroxy benzoic acid. 60

13. Artificial yarns and filaments of cellulose acetate containing olive oil and the methyl ester of para hydroxy benzoic acid.

14. Artificial yarns and filaments of cellulose acetate containing olive oil and the propyl ester 65 of para hydroxy benzoic acid.

15. Process of improving the properties of filaments or yarns containing cellulose acetate comprising applying thereto a finish containing a fatty material selected from the group consisting 70 of higher fatty acids and their glycerides and the methyl ester of a para hydroxy benzoic acid.

16. Process of improving the properties of filaments or yarns containing cellulose acetate comprising applying thereto a finish containing a 75

fatty material selected from the group consisting of higher fatty acids and their glycerides and the propyl ester of a para hydroxy benzoic acid.

17. Artificial material of cellulose acetate containing a fatty material selected from the group consisting of higher fatty acids and their glycerides and the methyl ester of a para hydroxy benzoic acid.

18. Artificial material of cellulose acetate containing a fatty material selected from the group consisting of higher fatty acids and their glycerides and the propyl ester of a para hydroxy benzoic acid.

5

GEORGE SCHNEIDER.